

No. 874,877.

PATENTED DEC. 24, 1907.

H. G. UNDERWOOD.  
METHOD OF CASTING.  
APPLICATION FILED JAN. 26, 1904.



# UNITED STATES PATENT OFFICE.

HERBERT GEORGE UNDERWOOD, OF STAMFORD, CONNECTICUT.

## METHOD OF CASTING.

No. 874,877.

Specification of Letters Patent.

Patented Dec. 24, 1907.

Application filed January 26, 1904. Serial No. 190,669.

*To all whom it may concern:*

Be it known that I, HERBERT GEORGE UNDERWOOD, a citizen of the United States, and a resident of Stamford, county of Fairfield, State of Connecticut, have invented 5 certain new and useful Improvements in Methods of Casting, of which the following is a description, reference being had to the accompanying drawing, in which the figure is a 10 longitudinal section of a casting apparatus such as may be used for the carrying out of my method and such as is more fully described and claimed in an application for patent filed on the same date as this.

15 While for clearness I illustrate my method by reference to a drawing of a particular form of casting apparatus, it will be understood that I may use any other construction capable of carrying out my method.

20 Heretofore the operation of casting as ordinarily practiced where the metal flows merely by gravity or is poured into ordinary molds, has been attended with a number of disadvantages. In order to get the metal to flow 25 freely it must be raised to a degree of heat much above the freezing point. This—particularly with alloys—tends to drive off some of the most important elements or constituents in the form of gas, and further tends to 30 “kill” the molten metal, and render a casting made therefrom weak and brittle. It is therefore detrimental to perfect casting that the metal in the melting pot should be raised to a temperature above the fusing point.

35 Again, where the molten metal is taken from a furnace into a ladle, and the ladle moved to a distant part of the casting room, it is necessary in order that the metal may retain enough heat to flow freely from the ladle, 40 that it be very highly heated at first and such heating as above stated takes away from the strength of the casting. Furthermore the loss of important constituents of the metal through over heating not only renders the resultant casting weak but such over heated metal continues to give forth gas even in the mold itself, and such gas unless it escapes 45 through the vents of the mold causes bubbles and blow holes in the casting. Also under

50 the common gravity system of casting and even under pressure system, there is always more or less air confined in the mold itself and unable to escape, which prevents the metal completely and sharply filling the mold 55 in all its angles and contours. When the

metal is forced into the mold as by a plunger, though the resultant casting is much better than under the ordinary gravity method, yet great care must be taken in placing the vents, as the whirling inrush of the metal into the 60 mold tends to close the vents before the gases and inclosed air can escape. Again, plungers or other mechanical devices moving in the molten metal to force it into the mold, tend to chill the metal and to become clogged, or if 65 the metal be raised to a very high degree of heat such as is necessary in alloys containing a large percentage of aluminium, to the casting of which my process is intended particularly to be applied, such moving parts become 70 melted before the metal is in condition for casting. It is necessary then in order to make a perfect casting at a high temperature, that the air be exhausted from the mold on all sides and that the forcing of the intensely 75 heated metal into the mold be done by some means not mechanical.

My method of casting does away with these disadvantages and a casting made in accordance therewith is much denser and 80 more homogeneous in mass and much sharper and cleaner in surface than ordinary castings.

Broadly my invention has for its main feature the exhausting of the air from the 85 mold and forcing the metal into said mold at the same time by compressed air, and in carrying out my method I can use such an apparatus as illustrated in the drawing where A indicates a melting furnace heat- 90 ed by ordinary means such as air and gas inlet B.

Supported in the furnace is the melting pot C having a forwardly projecting nozzle or mouth D and outlet port E which coincides with the inlet in the face plate of a mold containing chamber F which is supported on tracks G, H so as to move across the face of the nozzle E and thus bring the outlet and inlet ports into or out of coincidence with each other and thereby close or open the outlet E. As far as the main feature of my method goes however it is only necessary that there be a connection between the melting pot and the mold. 100

The chamber F contains the mold I held in place thereby by any suitable means as a bridge-clamp J. The mold may be provided with venting openings i though this is not necessary in a mold made in sections. The 110

chamber F has a cover K held in place by any appropriate fastening device, such as the bridge clamp L and from the chamber runs a pipe M which communicates by means 5 of a valve m either with the air or with an exhaust pipe O which is connected to any air exhausting apparatus. By means of this pipe air may be exhausted from the chamber and from the contained mold. 10 The extension of this pipe is shown in dotted lines 3.

The top of the melting pot C is closed and provided with any suitable cover P held in place thereon, and entering into said melting 15 pot above the surface of the metal therein is an air pipe R opening to the outside air or attached to a compressing apparatus or some source of compressed air, whereby the said air will force the metal in the pot into 20 the mold when the port E is opened.

The application of my method is as follows. After the metal is brought to a proper temperature in a melting pot, the air is exhausted in the mold-containing chamber. 25 The said chamber is then moved until its inlet and the mold inlet co-incide with the outlet from the melting pot and the metal having no impediment before it, and forced by pressure of the compressed air behind it, 30 is sucked and forced in, completely and entirely filling the mold in its smallest part or sharpest angle, and this with a fluidity of metal far less than ordinarily necessary.

It is absolutely requisite when a sand mold 35 is used that it be contained in a vacuum chamber, as by no other means can complete exhaustion of the air be accomplished, as, if the air be exhausted from one point only and not over the entire surface of the mold, the 40 porosity of the mold admits air as fast as it is exhausted, thus preventing the formation of a complete vacuum. In addition to this necessity of complete exhaustion there is also a great advantage in casting in a sand 45 mold surrounded by a vacuum chamber, as thereby the inflowing metal is drawn to all parts of the mold equally.

I have found that it is not necessary to do more than charge the melting pot once with 50 compressed air as the gases given off by the molten metal will keep up sufficient degree of compression when the surface of the metal is lowered. This is of advantage in that continued oxidation by the admission of fresh 55 air is obviated.

By using compressed air as a means of forcing the metal into the mold, I get a uniform pressure over the whole surface of the metal and also I do away with any mechanical parts moving in the metal and liable to 60 clog.

As before stated I show the casting apparatus of the drawing merely by way of illustration, and do not wish to have my method 65 in any way limited in its application either

as to the material to be cast, or the apparatus used—the essential feature of my invention being capable of being applied in a variety of ways and to casting from ladles, or dippers as well as directly from a melting 70 pot. Neither do I wish to be limited to any special degree of temperature or fluidity in the metal by the term molten as the degree necessary to make a casting depends upon varying conditions. 75

Having described my invention what I claim is—

1. A method of casting which consists in compressing the air above the surface of an inclosed mass of molten metal, and maintaining said pressure therein without forcing additional air therein exhausting the air from the interior of a mold, and opening connection between said mold and the metal whereby the molten metal will be forced and drawn 85 into the mold by both pressure and exhaustion, substantially as described.

2. A method of casting which consists in compressing the air above the surface of an inclosed mass of molten metal, and maintaining said air under pressure therein without forcing additional air above the surface of the inclosed metal inclosing a mold in an inclosed chamber, exhausting the air from the interior of the chamber and therefore 90 from its contained mold, opening connection between said mold and the molten metal and thereby forcing the metal into the mold, substantially as described. 95

3. A method of casting which consists in sealing a metal pot or other receptacle containing metal from outside air, charging the space above the metal with a compressed gas and cutting off the supply of gas until the melted metal has been forced from the melting pot, thus preventing continued oxidation 105 of the metal in the pot.

4. A method of casting which consists in sealing a melting pot or other receptacle containing molten metal from outside air, charging the space above the molten metal with compressed air, and cutting off the supply of compressed air until all the metal has been forced from the melting pot, thus preventing continued oxidation of the metal in the pot, 110 substantially as described.

5. A method of casting which consists in sealing from out-side air a melting pot or other receptacle containing metal to be melted and cast, charging the space above the metal with a compressed gas, cutting off the supply of gas, exhausting air from a mold and bringing the exhausted mold into communication with the sealed melting pot, whereby the metal will be drawn and forced 115 from said melting pot into the mold.

6. A method of casting which consists in sealing a melting pot or other receptacle containing molten metal from outside air, charging the space above the molten metal with 120

compressed air, and cutting off the supply of compressed air until the metal has been forced from the melting pot, thus preventing continued oxidation of the metal in the pot,  
5 exhausting air from the mold and bringing the exhausted mold into communication with the bottom of the melting pot whereby

the molten metal will be forced and drawn from the melting pot into the exhausted mold.

Witnesses:

HERBERT GEORGE UNDERWOOD.  
W. H. RUBY,  
F. B. WRIGHT.